

# UNITED STATES PATENT OFFICE.

WILLIAM M. JONES, OF SAN FRANCISCO, CALIFORNIA.

## LUBRICANT FOR COMMUTATORS.

SPECIFICATION forming part of Letters Patent No. 680,155, dated August 6, 1901.

Application filed January 7, 1901. Serial No. 42,424. (No specimens.)

*To all whom it may concern:*

Be it known that I, WILLIAM M. JONES, a citizen of the United States, residing at San Francisco, in the county of San Francisco and 5 State of California, have invented certain new and useful Improvements in Lubricants for Commutators, of which the following is a specification.

My invention relates to improvements in 10 lubricating compounds more especially intended for use on commutators, the object of my invention being to provide a commutator compound which will prevent sparking at the brushes and will also prevent the cutting of 15 the brushes and commutators.

In preparing this compound I take five pounds of paraffin-wax and three pounds of graphite and boil them together for about one hour and a half at a very high temperature. I have not been able to ascertain the 20 degree of such temperature; but it is as high a temperature as is possible without burning. In other words, the temperature must be maintained below that of spontaneous ignition. I find that during the process of boiling a heavy black smoke is given off for an 25 hour or more. The mixture then boils quite colorless without giving off any smoky vapor, and after boiling clear for fifteen or twenty minutes the boiling is stopped. It is found that the volume of the material has diminished quite an appreciable extent during the boiling. After the mixture has cooled a trifle I add about one teaspoonful of spermaceti. The mixture is then cooled in molds 30 in the form of sticks of suitable size and shape for the purpose desired.

In my experiments to provide a compound

which will prevent sparks I found that paraffin and graphite if mixed together without 40 boiling make a plastic compound which lubricates the commutator, but creates a great deal of sparking at the brushes. This sparking is no doubt due to the substance which is given off in the form of heavy black smoke, 45 before referred to, for I find that after this substance has been removed there is practically no sparking except that which is occasioned by pits or other defects in the commutators. I have also found that if the mixture 50 so boiled be cooled without the addition of the spermaceti the compound when solidified is no longer plastic, but is very brittle, and indeed has so little adhesiveness that it will not stay on the commutator. The addition of the small quantity of spermaceti gives 55 it sufficient adhesiveness to enable it to stick to the commutator. The lubricant will be found to color the commutator a light walnut color, and the surface of the commutator will 60 be polished.

I claim—

A solid lubricant comprising paraffin and graphite in substantially the proportions specified, which has been boiled at a high 65 temperature until the vapor driven off is perfectly colorless, to which a small quantity of spermaceti has been added after boiling and before cooling, substantially as described.

In witness whereof I have hereunto set my 70 hand in the presence of two subscribing witnesses.

W. M. JONES.

Witnesses:

FRANCIS M. WRIGHT,  
K. LOCKWOOD NEVINS.